# EUROPEAN PATENT SPECIFICATION

(11) **EP 2 010 632 B1**
(45) Date of publication and mention of the grant of the patent: **15.01.2020**
(21) Application number: 07760438.7
(22) Date of filing: 11.04.2007
(51) Int. Cl.: C10M 141/06

(54) **A METHOD FOR LUBRICATING A TRANSMISSION**
VERFAHREN ZUM SCHMIEREN EINES GETRIEBES
PROCÉDÉ DE LUBRIFICATION DE TRANSMISSION

(30) Priority: 12.04.2006 US 744671 P
(43) Date of publication of application: 07.01.2009
(73) Proprietor: The Lubrizol Corporation, Wickliffe, Ohio 44092 (US)
(72) Inventor: TIPTON, Craig D., Wickliffe, OH 44092 (US); BAKER, Mark R., Wickliffe, OH 44092 (US); LAHIRI, Shreyasi, Wickliffe, OH 44092 (US); ABRAHAM, William D., Wickliffe, OH 44092 (US); VICKERMAN, Richard J., Wickliffe, OH 44092 (US); PATTERSON, Suzanne M., Wickliffe, OH 44092 (US)
(74) Representative: D Young & Co LLP
(86) International application number: PCT/US2007/066371
(87) International publication number: WO 2007/121205

(56) References cited:
- EP-A- 0 919 605
- EP-A- 1 233 054
- EP-A1- 0 765 929
- GB-A- 1 222 169

## Description

### BACKGROUND OF THE INVENTION

The present invention relates to a method for lubricating a transmission.

In the automatic transmission marketplace, where there is rapid engineering change driven by the desire to reduce weight and increase transmission capacity, there is a desire for automatic transmission fluids that exhibit a high static coefficient of friction for improved clutch holding capacity. At the same time, there is a desire to improve the retention of positive slope characteristics in the µ/v (coefficient of friction vs. sliding speed) curve. There are newer tests in the marketplace which are used to define these characteristics. The static torque can be measured in tests such as the Toyota SAE#2 friction test procedure and the retention of positive slope can be measured by procedures like the JASO LVFA (Japan Automotive Standards Organization, Low Velocity Friction Apparatus) in which the slope of the µ/v curve is periodically measured during oxidative and mechanical aging.

There are patents, for example, US 5,750,476, where a type of friction modifier technology used to achieve this performance is described. The combined requirements of high static coefficient of friction and durable positive slope are often incompatible with traditional ATF friction modifier technology which is extremely well described in the patent literature. Many of the commonly used friction modifiers result in a low static coefficient of friction and are not durable enough on positive slope to be of sufficient use. Additional patent literature describing technology for retaining positive mu/v or anti-shudder characteristics include US 5,858,929. These may employ metal detergents and combinations of friction modifiers.

PCT Publication WO04/007652, Adams et al, January 22, 2004, discloses a fluid composition of (a) a friction modifier derived from the reaction of a carboxylic acid with an amino alcohol, the friction modifier containing at least two hydrocarbyl groups, and (b) a dispersant, which provides good friction properties in an automatic transmission.

U.S. Patent 4,886,612 discloses a lubricating oil comprising at least one of various products, which can be various imidazolines or an oxazoline of the structure where R₂ and R₃ each represent CH₂OCOR₁, CH₂OH or H, prepared by the condensation a carboxylic acid (or a reactive equivalent thereof) with an amino alcohol; for example, the condensation of two moles of isostearic acid with one mole of tris-hydroxymethylaminomethane (THAM).

EP 0 919 605 A discloses an automatic transmission fluid composition comprising (1) a major amount of a base oil and (2) a minor amount of an additive composition comprising: (A) a nitrogen- and phosphorous dispersant in which the total nitrogen to phosphorous mass ratio is between 3:1 and 10:1 and (B) at least one friction modifier.

EP 0 765 929 A discloses an additive for lubricating oils for diesel engines, comprising one or more kinds of amino alcohols which have one or more amino groups and one or more hydroxyl groups in a molecule and possess a function of dispersing water-containing calcium sulphate in oil, the hydroxyl groups being bound to the carbon atoms at the β-positions to the amino groups; and a lubricating oil composition for diesel engines, which comprises the additives in an amount of from 0.1 to 10 % by weight.

The present invention solves the problem of developing new and relatively simple and inexpensive friction modifiers to obtain high static coefficients of friction and maintain a durable positive slope during oxidative and mechanical stressing of the friction system, particularly for use in an automatic transmission. This is accomplished by the use of a friction modifier which comprises a tertiary amine having at least two alkyl groups of at least 6 carbon atoms, as further described below.

### SUMMARY OF THE INVENTION

The present invention provides a method for lubricating a transmission, comprising supplying thereto a lubricant comprising: (a) a major amount of an oil of lubricating viscosity; (b) 0.01 to 10 percent by weight of a tertiary amine being represented by the formula R¹R²NR³ wherein R¹ and R² are each independently an alkyl group of at least 6 carbon atoms and R³ is a polyhydroxyl-containing alkyl group or a polyhydroxyl-containing alkoxy alkyl group; and (c) 0.3 to 10 percent by weight of a dispersant.

### DETAILED DESCRIPTION OF THE INVENTION

Various preferred features and embodiments will be described below by way of non-limiting illustration.

One component used in the present invention is an oil of lubricating viscosity, which can be present in a major amount, for a lubricant composition, or in a concentrate forming amount, for a concentrate. Suitable oils include natural and synthetic lubricating oils and mixtures thereof. In a fully formulated lubricant, the oil of lubricating viscosity is generally present in a major amount (i.e. an amount greater than 50 percent by weight). Typically, the oil of lubricating viscosity is present in an amount of 75 to 95 percent by weight, and often greater than 80 percent by weight of the composition. For concentrates, the oil of lubricating viscosity may be present at lower concentration or in a minor amount, for example, from 10 to 50% by weight, and in one embodiment 10 to 30% by weight.

Natural oils useful in making the lubricants and functional fluids used in the invention include animal oils and vegetable oils as well as mineral lubricating oils such as liquid petroleum oils and solvent-treated or acid-treated mineral lubricating oils of the paraffinic, naphthenic or mixed paraffinic/-naphthenic types which may be further refined by hydrocracking and hydrofinishing processes.

Synthetic lubricating oils include hydrocarbon oils and halo-substituted hydrocarbon oils such as polymerized and interpolymerized olefins, also known as polyalphaolefins; polyphenyls; alkylated diphenyl ethers; alkyl-or dialkylbenzenes; and alkylated diphenyl sulfides; and the derivatives, analogs and homologues thereof. Also included are alkylene oxide polymers and inter-polymers and derivatives thereof, in which the terminal hydroxyl groups may have been modified by esterification or etherification. Also included are esters of dicarboxylic acids with a variety of alcohols, or esters made from C5 to C12 monocarboxylic acids and polyols or polyol ethers. Other synthetic oils include silicon-based oils, liquid esters of phosphorus-containing acids, and polymeric tetrahydrofurans. The synthetic oils may be produced by Fischer-Tropsch reactions and typically may comprise hydroisomerized Fischer-Tropsch hydrocarbons and/or waxes, or hydroisomerized slack waxes.

Unrefined, refined and rerefined oils, either natural or synthetic, can be used in the lubricants useful in the present invention. Unrefined oils are those obtained directly from a natural or synthetic source without further purification treatment. Refined oils have been further treated in one or more purification steps to improve one or more properties. They can, for example, be hydrogenated, resulting in oils of improved stability against oxidation.

In one embodiment, the oil of lubricating viscosity is an API Group II, Group III, Group IV, or Group V oil, including a synthetic oil, or mixtures thereof. These are classifications established by the API Base Oil Interchangeability Guidelines. Both Group II and Group III oils contain < 0.03 percent sulfur and > 99 percent saturates. Group II oils have a viscosity index of 80 to 120, and Group III oils have a viscosity index > 120. Polyalphaolefins are categorized as Group IV. Group V is encompasses "all others" (except for Group I, which contains > 0.03% S and/or < 90% saturates and has a viscosity index of 80 to 120).

In one embodiment, at least 50% by weight of the oil of lubricating viscosity is a polyalphaolefin (PAO). Typically, the polyalphaolefins are derived from monomers having from 4 to 30, or from 4 to 20, or from 6 to 16 carbon atoms. Examples of useful PAOs include those derived from 1-decene. These PAOs may have a viscosity of 1.5 to 150 mm²/s (cSt) at 100°C. PAOs are typically hydrogenated materials.

The oils useful in the present invention can encompass oils of a single viscosity range or a mixture of high viscosity and low viscosity range oils. In one embodiment, the oil exhibits a 100°C kinematic viscosity of 1 or 2 to 8 or 10 mm²/sec (cSt). The overall lubricant composition may be formulated using oil and other components such that the viscosity at 100°C is 1 or 1.5 to 10 or 15 or 20 mm²/sec and the Brookfield viscosity (ASTM-D-2983) at -40°C is less than 20 or 15 Pa-s (20,000 cP or 15,000 cP), such as less than 10 Pa-s, even 5 or less.

Component (b) is a tertiary amine, which can serve as a friction modifier. The amine will contain three substituent hydrocarbyl groups, two of which arc alkyl groups. The amine is represented by the formula

R¹R²NR³

wherein R¹ and R² are each independently an alkyl group of at least 6 carbon atoms (e.g., 8 to 20 carbon atoms or 10 to 18 or 12 to 16) and R³ is a polyhydroxyl-containing alkyl group or a polyhydroxyl-containing alkoxyalkyl group

In one embodiment the amine comprises a product of di-cocoalkyl amine or homologous amines. Di-cocoalkyl amine (or di-cocoamine) is a secondary amine in which two of the R groups in the above formula are predominantly C₁₂ groups, derived from coconut oil and the remaining R group is H.

In one embodiment, R³ is a polyol-containing alkyl group (that is, a group containing 2 or more hydroxy groups) or a group containing one or more hydroxy groups and one or more amine groups. For instance, R³ may be -CH₂-CHOH-CH₂OH or a homologue thereof, containing, for example, 3 to 8 carbon atoms or 3 to 6 carbon atoms or 3 to 4 carbon atoms, and 2, 3, 4 or more hydroxy groups (normally no more than one hydroxy group per carbon atom). A typical resulting product may thus be represented by

R¹R²N-CH₂-CHOH-CH₂OH

or homologues thereof, where R¹ and R² are, as described above, independently alkyl groups of 8 to 20 carbon atoms. Such products may be obtained by the reaction of a dialkyl amine with an epoxide or chlorohydroxy compound. In particular, reaction of a secondary amine with glycidol (2,3-epoxy-1-propanol) or "chloroglycerine" (that is, 3-chloropropane-1,2-diol) may be effective under conditions as described above. Such materials based on the reaction of dicocoamine with one or more moles of glycidol or chloroglycerine are particularly useful in providing friction-modifying performance. If reaction is with multiple moles of glycidol or chloroglycerine, or other epoxyalkanols or chlorodiols, a dimeric or oligomeric ether-containing group, that is, a hydroxyl-substituted alkoxyalkyl group, may result.

The amine, component (b), may alternatively be described, in certain embodiments, as a compound comprising a core portion comprising 3 to 8 carbon atoms, (e.g, 3 to 6, or 3 carbon atoms), said core portion being substituted by: (i) at least two hydroxy groups, or at least one hydroxy group and at least one alkoxy group of 1 to 4 carbon atoms wherein said alkoxy group is further substituted by at least one hydroxy group or another such alkoxy group; and (ii) at least one amino group, the nitrogen atom thereof bearing two hydrocarbyl groups, each such hydrocarbyl group independently having 6 to 30 carbon atoms.

The amount of component (b) in the compositions useful in the present invention is generally an amount suitable to reduce or inhibit shudder in an automatic transmission, that is, a performance defect observed during wet clutch operation when the friction characteristics of the transmission fluid are inadequately balanced. The effective amount is 0.01 to 10.0 percent by weight of the finished fluid formulation. Alternative amounts include 0.02 percent to 5 percent, or 0.1 percent to 3 percent, or 0.1 to 2 percent, or 0.5 to 1.5 percent. In a concentrate, the amounts will be proportionately higher.

Component (c) of the lubricant is a dispersant. It may be described as "other than a species of (b)," in the event that some of the friction modifiers of (b) may exhibit some dispersant characteristics. Examples of "carboxylic dispersants" are described in many U.S. Patents including the following: 3,219,666, 3,316,177, 3,340,281, 3,351,552, 3,381,022, 3,433,744, 3,444,170, 3,467,668, 3,501,405, 3,542,680, 3,576,743, 3,632,511, 4,234,435, Re 26,433, and 6,165,235.

Succinimide dispersants, a species of carboxylic dispersants, are prepared by the reaction of a hydrocarbyl-substituted succinic anhydride (or reactive equivalent thereof, such as an acid, acid halide, or ester) with an amine, as described above. The hydrocarbyl substituent group generally contains an average of at least 8, or 20, or 30, or 35 up to 350, or to 200, or to 100 carbon atoms. In one embodiment, the hydrocarbyl group is derived from a polyalkene. Such a polyalkene can be characterized by an M̅ₙ (number average molecular weight) of at least 500. Generally, the polyalkene is characterized by an M̅ₙ of 500, or 700, or 800, or 900 up to 5000, or to 2500, or to 2000, or to 1500. In another embodiment M̅ₙ varies from 500, or 700, or 800, to 1200 or 1300. In one embodiment the polydispersity (M̅_{w}/M̅ₙ) is at least 1.5.

The polyalkenes include homopolymers and inter-polymers of polymerizable olefin monomers of 2 to 16 or to 6, or to 4 carbon atoms. The olefins may be monoolefins such as ethylene, propylene, 1-butene, isobutene, and 1-octene; or a polyolefinic monomer, such as diolefinic monomer, such 1,3-butadiene and isoprene. In one embodiment, the inter-polymer is a homopolymer. An example of a polymer is a polybutene. In one instance about 50% of the polybutene is derived from isobutylene. The polyalkenes can be prepared by conventional procedures.

In one embodiment, the succinic acylating agents are prepared by reacting a polyalkene with an excess of maleic anhydride to provide substituted succinic acylating agents wherein the number of succinic groups for each equivalent weight of substituent group is at least 1.3, e.g., 1.5, or 1.7, or 1.8. The maximum number of succinic groups per substituent group generally will not exceed 4.5, or 2.5, or 2.1, or 2.0. The preparation and use of substituted succinic acylating agents wherein the substituent is derived from such polyolefins are described in U.S. Patent 4,234,435.

The substituted succinic acylating agent can be reacted with an amine, including those amines described above and heavy amine products known as amine still bottoms. The amount of amine reacted with the acylating agent is typically an amount to provide a mole ratio of CO:N of 1:2 to 1:0.75, . If the amine is a primary amine, complete condensation to the imide can occur. Varying amounts of amide product, such as the amidic acid, may also be present. If the reaction is, rather, with an alcohol, the resulting dispersant will be an ester dispersant. If both amine and alcohol functionality are present, whether in separate molecules or in the same molecule (as in the above-described condensed amines), mixtures of amide, ester, and possibly imide functionality can be present. These are the so-called ester-amide dispersants.

"Amine dispersants" are reaction products of relatively high molecular weight aliphatic or alicyclic halides and amines, such as polyalkylene polyamines. Examples thereof are described in the following U.S. Patents: 3,275,554, 3,438,757, 3,454,555, and 3,565,804.

"Mannich dispersants" are the reaction products of alkyl phenols in which the alkyl group contains at least 30 carbon atoms with aldehydes (especially formaldehyde) and amines (especially polyalkylene polyamines). The materials described in the following U.S. Patents are illustrative: 3,036,003, 3,236,770, 3,414,347, 3,448,047, 3,461,172, 3,539,633, 3,586,629, 3,591,598, 3,634,515, 3,725,480, 3,726,882, and 3,980,569.

Post-treated dispersants are also part of the present invention. They are generally obtained by reacting at carboxylic, amine or Mannich dispersants with reagents such as urea, thiourea, carbon disulfide, aldehydes, ketones, carboxylic acids, hydrocarbon-substituted succinic anhydrides, nitriles, epoxides, boron compounds such as boric acid (to give "borated dispersants"), phosphorus compounds such as phosphorus acids or anhydrides, or 2,5-dimercaptothiadiazole (DMTD). Exemplary materials of this kind are described in the following U.S. Patents: 3,200,107, 3,282,955, 3,367,943, 3,513,093, 3,639,242, 3,649,659, 3,442,808, 3,455,832, 3,579,450, 3,600,372, 3,702,757, and 3,708,422. Other related dispersants include composition comprising the product prepared by heating together: (a) a dispersant as described above and (b) 2,5-dimercapto-1,3,4-thiadiazole or a hydrocarbyl-substituted 2,5-dimercapto-1,3,4-thiadiazole which is substantially insoluble in a hydrocarbon oil of lubricating viscosity at 25°C, and further either (c) a borating agent or (d) an inorganic phosphorus compound, or both (c) and (d), said heating being sufficient to provide a reaction product of (a), (b), and (c) or (d) which is soluble in said hydrocarbon oil at 25°C. These materials are described in US Application 2005-0041395.

Mixtures of dispersants can also be used.

The amount of component (c) in the compositions useful in the present invention is 0.3 to 10 percent by weight. In other embodiments, the amount of component (c) is 0.5 to 7 percent or 1 to 5 percent of the final blended fluid formulation. In a concentrate, the amounts will be proportionately higher.

Other components which are conventionally employed in a transmission fluid, in particular, and automatic transmission fluid (ATF) are typically also present.

The functional fluid may contain one or more viscosity modifiers and/or dispersant viscosity modifiers. Viscosity modifiers (VM) and dispersant viscosity modifiers (DVM) are well known. Examples of VMs and DVMs include polymethacrylates, polyacrylates, polyolefins, styrene-maleic ester copolymers, and similar polymeric substances including homopolymers, copolymers and graft copolymers. The DVM may comprise a nitrogen-containing methacrylate polymer, for example, a nitrogen-containing methacrylate polymer derived from methyl methacrylate and dimethylaminopropyl amine.

Examples of commercially available VMs, DVMs and their chemical types include the following: polyisobutylenes (such as Indopol™ from BP Amoco or Parapol™ from ExxonMobil); olefin copolymers (such as Lubrizol™ 7060, 7065, and 7067 from Lubrizol and Lucant™ HC-2000L and HC-600 from Mitsui); hydrogenated styrene-diene copolymers (such as Shellvis™ 40 and 50, from Shell and LZ® 7308, and 7318 from Lubrizol); styrene/maleate copolymers, which are dispersant copolymers (such as LZ® 3702 and 3715 from Lubrizol); polymethacrylates, some of which have dispersant properties (such as those in the Viscoplex™ series from RohMax, the Hitec™ series from Afton, and LZ 7702™, LZ 7727™, LZ 7725™ and LZ 7720C™ from Lubrizol); olefingraft-polymethacrylate polymers (such as Viscoplex™ 2-500 and 2-600 from RohMax); and hydrogenated polyisoprene star polymers (such as Shellvis™ 200 and 260, from Shell). Viscosity modifiers that may be used are described, for instance, in U.S. patents 5,157,088, 5,256,752 and 5,395,539. The VMs and/or DVMs may be used in the functional fluid at a concentration of up to 20% by weight. Concentrations of 1 to 12%, or 3 to 10% by weight may be used.

Another component that may be used in the composition used in the present invention is a supplemental friction modifier. Friction modifiers are well known to those skilled in the art. A useful list of friction modifiers is included in U.S. Pat. No. 4,792,410. U.S. Patent 5,110,488 discloses metal salts of fatty acids and especially zinc salts, useful as friction modifiers. A list of friction modifiers includes:
(i) fatty phosphites
(ii) fatty acid amides
(iii) fatty epoxides
(iv) borated fatty epoxides
(v) fatty amines other than component (b) above
(vi) glycerol esters, e.g., partial esters
(vii) borated glycerol esters
(viii) alkoxylated fatty amines
(ix) borated alkoxylated fatty amines
(x) metal salts of fatty acids
(xi) sulfurized olefins
(xii) fatty imidazolines
(xiii) condensation products of carboxylic acids and polyalkylenepolyamines
(xiv) metal salts of alkyl salicylates
(xv) amine salts of alkylphosphoric acids
(xvi) ethoxylated alcohols
and mixtures thereof.

Representatives of each of these types of friction modifiers are known and are commercially available. For instance, (i) fatty phosphites are generally of the formula (RO)₂PHO. The dialkyl phosphite, as shown in the preceding formula, is typically present with a minor amount of monoalkyl phosphite of the formula (RO)(HO)PHO. In these structures, the term "R" is conventionally referred to as an alkyl group. It is, of course, possible that the alkyl is actually alkenyl and thus the terms "alkyl" and "alkylated," as used herein, will embrace other than saturated alkyl groups within the phosphite. The phosphite should have sufficient hydrocarbyl groups to render the phosphite substantially oleophilic. In one embodiment, the hydrocarbyl groups are substantially unbranched. Many suitable phosphites are available commercially and may be synthesized as described in U.S. Patent 4,752,416. The phosphite may contain 8 to 24 carbon atoms in each of R groups. In certain embodiments, the fatty phosphite contains 12 to 22 carbon atoms in each of the fatty radicals, alternatively 16 to 20 carbon atoms. In one embodiment the fatty phosphite can be formed from oleyl groups, thus having 18 carbon atoms in each fatty radical.

(iv) Borated fatty epoxides are known from Canadian Patent No. 1,188,704. These oil-soluble boron- containing compositions are prepared by reacting, at a temperature from 80°C to 250°C, boric acid or boron trioxide with at least one fatty epoxide having the formula wherein each of R¹, R², R³ and R⁴ is hydrogen or an aliphatic radical, or any two thereof together with the epoxy carbon atom or atoms to which they are attached, form a cyclic radical. The fatty epoxide may, in one embodiment, contain at least 8 carbon atoms.

The borated fatty epoxides can be characterized by the method for their preparation which involves the reaction of two materials. Reagent A can be boron trioxide or any of the various forms of boric acid including metaboric acid (HBO₂), orthoboric acid (H₃BO₃) and tetraboric acid (H₂B₄0₇). Boric acid, and especially orthoboric acid, may be used. Reagent B can be at least one fatty epoxide having the above formula. In the formula, each of the R groups is most often hydrogen or an aliphatic radical with at least one being a hydrocarbyl or aliphatic radical containing at least 6 carbon atoms. The molar ratio of reagent A to reagent B is generally 1:0.25 to 1:4. Ratios of 1:1 to 1:3 may be used, with about 1:2 being exemplary. The borated fatty epoxides can be prepared by merely blending the two reagents and heating them at temperature of 80° to 250°C, such as 100° to 200°C, for a period of time sufficient for reaction to take place. If desired, the reaction may be effected in the presence of a substantially inert, normally liquid organic diluent. During the reaction, water is evolved and may be removed by distillation.

(iii) Non-borated fatty epoxides, corresponding to "Reagent B" above, are also useful as friction modifiers.

Borated amines are generally known from U.S. Patent 4,622,158. Borated amine friction modifiers (including (ix) borated alkoxylated fatty amines) are conveniently prepared by the reaction of a boron compounds, as described above, with the corresponding amines. The amine can be a simple fatty amine or hydroxy containing tertiary amines. The borated amines can be prepared by adding the boron reactant, as described above, to an amine reactant and heating the resulting mixture at a 50° to 300°C, such as 100°C to 250°C or 150°C to 230°C, with stirring. The reaction is continued until by-product water ceases to evolve from the reaction mixture indicating completion of the reaction.

Among the amines useful in preparing the borated amines are commercial alkoxylated fatty amines known by the trademark "ETHOMEEN" and available from Akzo Nobel. Representative examples of these ETHOMEEN™ materials is ETHOMEEN™ C/12 (bis[2-hydroxyethyl]-coco-amine); ETHOMEEN™ C/20 (polyoxyethylene[10]cocoamine); ETHOMEEN™ S/12 (bis[2-hydroxyethyl]soyamine); ETHOMEEN™ T/12 (bis[2-hydroxyethyl]-tallow-amine); ETHOMEEN™ T/15 (polyoxyethylene-[5]tallowamine); ETHOMEEN™ 0/12 (bis[2-hydroxyethyl]oleyl-amine); ETHOMEEN™ 18/12 (bis[2-hydroxyethyl]octadecylamine); and ETHOMEEN™ 18/25 (polyoxyethyl-ene[15]octadecylamine). Fatty amines and ethoxylated fatty amines are also described in U.S. Patent 4,741,848.

The (viii) alkoxylated fatty amines, and (v) fatty amines themselves (such as oleylamine) are generally useful as friction modifiers in this invention. Such amines are commercially available.

Both borated and unborated fatty acid esters of glycerol can be used as friction modifiers. The (vii) borated fatty acid esters of glycerol are prepared by borating a fatty acid ester of glycerol with boric acid with removal of the water of reaction. In one embodiment, there is sufficient boron present such that each boron will react with from 1.5 to 2.5 hydroxyl groups present in the reaction mixture. The reaction may be carried out at a temperature in the range of 60°C to 135°C, in the absence or presence of any suitable organic solvent such as methanol, benzene, xylenes, toluene, or oil.

(vi) Fatty acid esters of glycerol themselves can be prepared by a variety of methods well known in the art. Many of these esters, such as glycerol monooleate and glycerol tallowate, are manufactured on a commercial scale. The esters useful are oil-soluble and may be prepared from C8 to C22 fatty acids or mixtures thereof such as are found in natural products and as are described in greater detail below. Fatty acid monoesters of glycerol are suitable, although, mixtures of mono- and diesters may be used. For example, commercial glycerol monooleate may contain a mixture of 45% to 55% by weight monoester and 55% to 45% diester.

Fatty acids can be used in preparing the above glycerol esters; they can also be used in preparing their (x) metal salts, (ii) amides, and (xii) imidazolines, any of which can also be used as friction modifiers. Suitable fatty acids include those containing 6 to 24 carbon atoms, or 8 to 18. The acids can be branched or straight-chain, saturated or unsaturated. Suitable acids include 2-ethylhexanoic, decanoic, oleic, stearic, isostearic, palmitic, myristic, palmitoleic, linoleic, lauric, and linolenic acids, and the acids from the natural products tallow, palm oil, olive oil, peanut oil, corn oil, and Neat's foot oil. A suitable acid is oleic acid.

Suitable metal salts of acids include zinc and calcium salts. Zinc salt of carboxylic acids, for instance. These zinc salts may be acidic, neutral or basic (overbased). These salts may be prepared from the reaction of a zinc containing reagent with a carboxylic acid or salt thereof. A useful method of preparation of these salts is to react zinc oxide with a carboxylic acid. Useful carboxylic acids are those described hereinabove, and include those of the formula RCOOH, where R is an aliphatic or alicyclic hydrocarbon radical. Also suitable are those wherein R is a fatty group, e.g., stearyl, oleyl, linoleyl, or palmityl. Also suitable are zinc salts wherein zinc is present in a stoichiometric excess over the amount needed to prepare a neutral salt. Such salts include those wherein the zinc is present from about 1.1 to about 1.8 times the stoichiometric, especially from 1.3 to 1.6 times the stoichiometric amount of zinc. These zinc carboxylates are known in the art and are described in U.S. Pat. 3,367,869. Certain basic zinc salts can be represented by the general formula Zn₄Oleate₆O₁. Metal salts may also include calcium salts, such as overbased calcium salts.

Suitable amides are those prepared by condensation of an acid with ammonia or with primary or secondary amines such as diethylamine and diethanolamine. Fatty imidazolines are the cyclic condensation product of an acid with a diamine or polyamine such as a polyethylenepolyamine. The imidazolines are generally represented by the structure where R is an alkyl group and R' is hydrogen or a hydrocarbyl group or a substituted hydrocarbyl group, including -(CH₂CH₂NH)n- groups. In one embodiment the friction modifier is the condensation product of a C8 to C24 fatty acid with a polyalkylene polyamine, and in particular, the product of isostearic acid with tetraethylenepentamine. The condensation products of carboxylic acids and polyalkyleneamines (xiii) may generally be imidazolines or amides.

Sulfurized olefins (xi) are well known commercial materials used as friction modifiers. A suitable sulfurized olefin is one which is prepared in accordance with the detailed teachings of U.S. Patents 4,957,651 and 4,959,168. Described therein is a cosulfurized mixture of 2 or more reactants selected from the group consisting of (1) at least one fatty acid ester of a polyhydric alcohol, (2) at least one fatty acid, (3) at least one olefin, and (4) at least one fatty acid ester of a monohydric alcohol.

Reactant (3), the olefin component, comprises at least one olefin. This olefin may be an aliphatic olefin, which usually will contain 4 to 40 carbon atoms, or 8 to 36 carbon atoms. Terminal olefins, or alpha-olefins, may be used, such as those having 12 to 20 carbon atoms. Mixtures of these olefins are commercially available, and such mixtures are contemplated for use in this invention.

The cosulfurized mixture of two or more of the reactants, is prepared by reacting the mixture of appropriate reactants with a source of sulfur. The mixture to be sulfurized can contain 10 to 90 parts of Reactant (1), or 0.1 15 parts by weight of Reactant (2); or 10 to 90 parts, often 15 to 60 parts, more often 25 to 35 parts by weight of Reactant (3), or 10 to 90 parts by weight of reactant (4). The mixture, in the present invention, includes Reactant (3) and at least one other member of the group of reactants identified as reactants (1), (2) and (4). The sulfurization reaction generally is effected at an elevated temperature with agitation and optionally in an inert atmosphere and in the presence of an inert solvent. The sulfurizing agents useful in the process of the present invention include elemental sulfur, hydrogen sulfide, sulfur halide plus sodium sulfide, and a mixture of hydrogen sulfide and sulfur or sulfur dioxide. Typically often 0.5 to 3 moles of sulfur are employed per mole of olefinic bonds.

Metal salts of alkyl salicylates (xiv) include calcium and other salts of long chain (e.g. C12 to C16) alkyl-substituted salicylic acids.

Amine salts of alkylphosphoric acids (xv) include salts of oleyl and other long chain esters of phosphoric acid, with amines as described below. Useful amines in this regard are tertiary-aliphatic primary amines, sold under the tradename Primene™. The supplemental friction modifier can be used in addition to component (a). The amount of the supplemental friction modifier is generally 0.1 to 1.5 percent by weight of the lubricating composition, such as 0.2 to 1.0 or 0.25 to 0.75 percent. In some embodiments, however, the amount of the supplemental friction modifier is present at less than 0.2 percent or less than 0.1 percent by weight, for example, 0.01 to 0.1 percent. In one embodiment the amount of bis-(2-hydroxyethyl)tallowamine (commercially sold as Ethomeen-12™) in particular is restricted to these low amounts or less.

Yet other suitable friction modifiers include friction modifiers derived from the reaction of a carboxylic acid or a reactive equivalent thereof with an aminoalcohol, wherein the friction modifier contains at least two hydrocarbyl groups, each containing at least 6 carbon atoms. Examples include the reaction product of isostearic acid or an alkyl succinic anhydride with tris-hydroxymethylaminomethane, which may be in a 2:1 mole ratio. These friction modifiers are described in greater detail in US Application 2005-0250655. Also suitable are amide or thioamide friction modifiers represented by the formula

R¹R²N-C(X)R³

wherein X is O or S. R¹ and R² may be hydrocarbyl groups of at least 6 carbon atoms, and R³ is a hydroxyalkyl group of 1 to 6 carbon atoms or a group formed by the condensation of said hydroxyalkyl group, through a hydroxyl group thereof, with an acylating agent. An example of such a friction modifier is the condensation product of dicocoamine with glycolic acid. These friction modifiers are described in greater detail in International application serial No. PCT/US 2006/039768, filed October 11, 2006. In certain embodiments, no (or less than 0.1%) additional friction modifier is present, other than that of component (b).

The compositions useful in the present invention can also include a detergent. Detergents as used herein are metal salts of organic acids. The organic acid portion of the detergent is a sulfonate, carboxylate, phenate, salicylate. The metal portion of the detergent is an alkali or alkaline earth metal. Suitable metals include are sodium, calcium, potassium and magnesium. Typically, the detergents are overbased, meaning that there is a stoichiometric excess of metal over that needed to form the neutral metal salt.

Suitable overbased organic salts include the sulfonate salts having a substantially oleophilic character and which are formed from organic materials. Organic sulfonates are well known materials in the lubricant and detergent arts. The sulfonate compound should contain on average 10 to 40 carbon atoms, such as 12 to 36 carbon atoms or 14 to 32 carbon atoms on average. Similarly, the phenates, salicylates, and carboxylates have a substantially oleophilic character.

While the present invention allows for the carbon atoms to be either aromatic or in paraffinic configuration, in certain embodiments alkylated aromatics are employed. While naphthalene based materials may be employed, the aromatic of choice is the benzene moiety.

A suitable composition is thus an overbased monosulfonated alkylated benzene, and may be the monoalkylated benzene. Typically, alkyl benzene fractions are obtained from still bottom sources and are mono- or dialkylated. It is believed, in the present invention, that the mono-alkylated aromatics may be superior to the dialkylated aromatics in overall properties.

It is desired that a mixture of mono-alkylated aromatics (benzene) be utilized to obtain the mono-alkylated salt (benzene sulfonate) in the present invention. The mixtures wherein a substantial portion of the composition contains polymers of propylene as the source of the alkyl groups assist in the solubility of the salt. The use of mono-functional (e.g., mono-sulfonated) materials avoids crosslinking of the molecules with less precipitation of the salt from the lubricant.

In certain embodiments, the salt may be "overbased." By overbasing, it is meant that a stoichiometric excess of the metal be present over that required to neutralize the anion of the salt. The excess metal from overbasing has the effect of neutralizing acids which may build up in the lubricant. A second advantage is that the overbased salt increases the dynamic coefficient of friction. Typically, the excess metal will be present over that which is required to neutralize the anion at in the ratio of up to 30:1, such as 5:1 to 18:1 on an equivalent basis.

The amount of the overbased salt utilized in the composition is typically 0.025 to 3 weight percent on an oil free basis, or 0.1 to 1.0 percent. The overbased salt is usually made up in about 50% oil with a TBN range of 10-600 on an oil free basis. Borated and non-borated overbased detergents are described in U.S. Patents 5,403,501 and 4,792,410.

The compositions useful in the present invention can also include at least one phosphorus acid, phosphorus acid salt, phosphorus acid ester or derivative thereof including sulfur-containing analogs in the amount of 0.002-1.0 weight percent. The phosphorus acids, salts, esters or derivatives thereof include phosphoric acid, phosphorous acid, phosphorus acid esters or salts thereof, phosphites, phosphorus-containing amides, phosphorus-containing carboxylic acids or esters, phosphorus-containing ethers, and mixtures thereof.

In one embodiment, the phosphorus acid, ester or derivative can be an organic or inorganic phosphorus acid, phosphorus acid ester, phosphorus acid salt, or derivative thereof. The phosphorus acids include the phosphoric, phosphonic, phosphinic, and thiophosphoric acids including dithiophosphoric acid as well as the monothiophosphoric, thiophosphinic and thiophosphonic acids. One group of phosphorus compounds are alkylphosphoric acid mono alkyl primary amine salts as represented by the formula where R¹, R², R³ are alkyl or hydrocarbyl groups or one of R¹ and R² can be H. The materials can be a 1:1 mixture of dialkyl and monoalkyl phosphoric acid esters. Compounds of this type are described in U.S. Patent 5,354,484.

Eighty-five percent phosphoric acid is a suitable material for addition to the fully-formulated compositions and can be included at a level of 0.01-0.3 weight percent based on the weight of the composition, such as 0.03 to 0.2 or to 0.1 percent.

Other materials can optionally be included in the compositions useful in the present invention, provided that they are not incompatible with the aforementioned required components or specifications. Such materials include antioxidants (that is, oxidation inhibitors), including hindered phenolic antioxidants, secondary aromatic amine antioxidants such as dinonyldiphenylamine as well as such well-known variants as monononyldiphenylamine and diphenylamines with other alkyl substituents such as mono- or di-ocyl, sulfurized phenolic antioxidants, oil-soluble copper compounds, phosphorus-containing antioxidants, and organic sulfides, disulfides, and polysulfides such as 2-hydroxyalkyl,alkyl thioethers or 1-t-dodecylthio-2-propanol or sulfurized 4-carbobutoxycyclohexene or other sulfurized olefins. Other optional components include seal swell compositions, such as isodecyl sulfolane or phthalate esters, which are designed to keep seals pliable. Also permissible are pour point depressants, such as alkylnaphthalenes, polymethacrylates, vinyl acetate/fumarate or /maleate copolymers, and styrene/maleate copolymers. Another material is an anti-wear agent such as zinc dialkyldithiophosphates. These optional materials are known to those skilled in the art, are generally commercially available, and are described in greater detail in published European Patent Application 761,805. Also included can be known materials such as corrosion inhibitors (e.g., tolyltriazole, dimercaptothiadiazoles), dyes, fluidizing agents, odor masking agents, and antifoam agents. Organic borate esters and organic borate salts can also be included.

The above components can be in the form of a fully-formulated lubricant or in the form of a concentrate within a smaller amount of lubricating oil. If they are present in a concentrate, their concentrations will generally be directly proportional to their concentrations in the more dilute form in the final blend.

### Examples

Lubricant formulations are prepared with the following components:

| Component\ Ex: | 1 | 2 | 3 | 4 | 5 | 6 | 7 | 8 | 9 | 10 |
|---|---|---|---|---|---|---|---|---|---|---|
| **DISPERSANTS** | | | | | | | | | | |
| Succinimide dispersant (including 40% oil) | 4.0 | 4.0 | 4.0 | 5.0 | 4.0 | 5.0 | | 4.5 | | |
| Succinimide Dispersant treated with DMTD^{b} (incl. 49% oil) | 1.0 | 1.0 | 1.0 | | 1.0 | | | 0.5 | | |
| Succinimide Dispersant treated with Boron (incl. 50% oil) | | | | 0.5 | | 0.5 | 5.0 | 0.5 | | |
| Succinimide Dispersant treated with TPA^{a} (including oil) | | | | | | | | | 5.0 | |
| Succinimide Dispersant treated with phosphorus and boron compounds (incl. oil) | | | | | | | | | | 5.0 |

| **AMINE** | | | | | | | | | | |
|---|---|---|---|---|---|---|---|---|---|---|
| Reaction product of Armeen 2C™ with 2,3-epoxy-1-propanol (1: 1 mole) | | | 0.5 | 0.5 | 0.5 | | | 0.8 | 0.8 | 0.8 |
| Reaction product of Armeen 2C™ with 3-chloropropane-1,2-diol (1:1 mole) | 1.25 | | | | | | | | | |
| Reaction product of Armeen™ HTL8^{c} with 2,3-epoxy-1-propanol (1:1 mole) | | 1.0 | | | | 1.25 | 1.25 | | | |

| **INHIBITORS** | | | | | | | | | | |
|---|---|---|---|---|---|---|---|---|---|---|
| 2-hydroxyalkyl,alkyl thioether | 0.5 | 0.5 | | | | 0.5 | | 0.5 | 0.5 | 0.5 |
| Dinonyldiphenylamine | 0.6 | 0.6 | 0.6 | 0.6 | | 0.6 | 0.8 | 0.6 | 0.6 | 0.6 |
| Hindered phenolic antioxidant | | | 0.5 | | | | | 0.5 | 0.5 | 0.5 |

| **FRICTION MODIFIERS** | | | | | | | | | | |
|---|---|---|---|---|---|---|---|---|---|---|
| Borate Ester | 0.2 | 0.2 | 0.2 | | | | | 0.2 | 0.2 | 0.2 |
| Diphenylphosphite | | | 0.25 | | | 0.25 | | | | |
| Dibutyl hydrogen phosphite | 0.11 | 0.11 | | 0.2 | | | 0.2 | 0.2 | 0.2 | 0.2 |
| Phosphoric acid | 0.1 | 0.1 | | 0.06 | | | 0.06 | 0.06 | 0.06 | 0.06 |

| **OTHERS** | | | | | | | | | | |
|---|---|---|---|---|---|---|---|---|---|---|
| Sulfolane seal swell agent | 0.4 | 0.4 | 0.4 | 0.35 | | 0.35 | 0.4 | 0.4 | 0.4 | 0.4 |
| Tolyltriazole | | | | 0.02 | | 0.02 | | 0.02 | 0.02 | 0.02 |
| Fatty carboxylic acid product with polyamine | | | | 0.1 | | | | 0.1 | 0.1 | 0.1 |
| Oil of lubricating viscosity^{d} | - balance - | | | | | | | | | |

| | | | | | | | | | | |
|---|---|---|---|---|---|---|---|---|---|---|
| a. Dispersant treated with terephthalic acid (TPA), optionally also treated with dimercaptothiadiazole, inorganic phosphorus acid, and/or boron b. DMTD = dimercaptothiadiazole c. secondary amine(s) having 2-ethylhexyl and hydrogenated tallow alkyl groups d. May include small amounts of other materials commonly present such as a viscosity index improver or an anti-foam agent. | | | | | | | | | | |

The friction modifier (a), used in combination with the dispersant (b) present in the base formulation, will provide good friction properties.

Unless otherwise indicated, each chemical or composition referred to herein should be interpreted as being a commercial grade material which may contain the isomers, by-products, derivatives, and other such materials which are normally understood to be present in the commercial grade. However, the amount of each chemical component is presented exclusive of any solvent or diluent oil, which may be customarily present in the commercial material, unless otherwise indicated.

## Claims

1. A method for lubricating a transmission, comprising supplying thereto a lubricant comprising:
(a) a major amount of an oil of lubricating viscosity;
(b) 0.01 to 10 percent by weight of a tertiary amine being represented by the formula
R¹R²NR³
wherein R¹ and R² are each independently an alkyl group of at least 6 carbon atoms and R³ is a polyhydroxyl-containing alkyl group or a polyhydroxyl-containing alkoxy alkyl group; and
(c) 0.3 to 10 percent by weight of a dispersant.

2. The method of claim 1 wherein the transmission is an automatic transmission.

3. The method of claim 1 wherein R¹ and R² are each independently alkyl groups of 8 to 20 carbon atoms.

4. The method of claim 1 wherein the tertiary amine is a product derived from di-cocoalkyl amine.

5. The method of claim 1 wherein R³ is a polyol-containing alkyl group.

6. The method of claim 1 wherein the amine of (b) is represented by the formula
R¹R²N-CH₂-CHOH-CH₂OH
wherein R¹ and R² are each independently alkyl groups of about 8 to about 20 carbon atoms.

7. The method of claim 1 wherein the amine of (b) comprises the reaction product of di-cocoamine and one or more moles of 2,3-epoxy-1- propanol or 3-chloropropane-1,2-diol.

8. The method of claim 1 wherein the dispersant comprises a succinimide dispersant.

9. The method of claim 1 wherein the lubricant further comprises at least one additive selected from the group consisting of detergents, antioxidants, seal swell agents, anti-wear agents, and friction modifiers.

10. The method of claim 1 wherein the lubricant further comprises at least one additive selected from the group consisting of organic borate esters organic borate salts, organic phosphorus esters, organic phosphorus salts, inorganic phosphorus acids, and inorganic phosphorus salts.

## Patentansprüche

1. Verfahren zum Schmieren eines Getriebes, bei dem man diesem eine Zusammensetzung zuführt, die Folgendes umfasst:
(a) eine größere Menge eines Öls mit Schmierviskosität;
(b) 0,01 bis 10 Gewichtsprozent eines tertiären Amins, das durch die Formel
R¹R²NR³
wiedergegeben wird, wobei R¹ und R² jeweils unabhängig für eine Alkylgruppe mit mindestens 6 Kohlenstoffatomen stehen und R³ für eine polyhydroxylgruppenhaltige Alkylgruppe oder eine polyhydroxylgruppenhaltige Alkoxyalkylgruppe steht; und
(c) 0,3 bis 10 Gewichtsprozent eines Dispergiermittels.

2. Verfahren nach Anspruch 1, wobei es sich bei dem Getriebe um ein Automatikgetriebe handelt.

3. Verfahren nach Anspruch 1, wobei R¹ und R² jeweils unabhängig für Alkylgruppen mit 8 bis 20 Kohlenstoffatomen stehen.

4. Verfahren nach Anspruch 1, wobei es sich bei dem tertiären Amin um ein von Dicocoalkylamin abgeleitetes Produkt handelt.

5. Verfahren nach Anspruch 1, wobei R³ für eine polyolhaltige Alkylgruppe steht.

6. Verfahren nach Anspruch 1, wobei das Amin (b) durch die Formel
R¹R²N-CH₂-CHOH-CH₂OH
wiedergegeben wird, wobei R¹ und R² jeweils unabhängig für Alkylgruppen mit etwa 8 bis etwa 20 Kohlenstoffatomen stehen.

7. Verfahren nach Anspruch 1, wobei das Amin von (b) das Reaktionsprodukt von Dicocoamin und einem oder mehreren Molen von 2,3-Epoxy-1-propanol oder 3-Chlorpropan-1,2-diol umfasst.

8. Verfahren nach Anspruch 1, wobei das Dispergiermittel ein Succinimid-Dispergiermittel umfasst.

9. Verfahren nach Anspruch 1, wobei das Schmiermittel mindestens ein Additiv aus der Gruppe bestehend aus Detergentien, Antioxidantien, Dichtungsquellmitteln, Verschleißschutzmitteln und Reibungsmodifikatoren umfasst.

10. Verfahren nach Anspruch 1, wobei das Schmiermittel ferner mindestens ein Additiv aus der Gruppe bestehend aus organischen Boratestern, organischen Boratsalzen, organischen Phosphorestern, organischen Phosphorsalzen, anorganischen Phosphorsäuren und anorganischen Phosphorsalzen umfasst.

## Revendications

1. Procédé de lubrification d'une transmission, comprenant l'apport à ladite transmission d'un lubrifiant comprenant :
(a) une quantité majeure d'une huile ayant une viscosité de lubrification ;
(b) 0,01 à 10 % en poids d'une amine tertiaire représentée par la formule
R¹R²NR³
dans laquelle R¹ et R² sont chacun indépendamment un groupe alkyle comportant au moins 6 atomes de carbone et R³ est un groupe alkyle contenant un groupe polyhydroxyle ou un groupe alcoxyalkyle contenant un groupe polyhydroxyle ; et
(c) 0,3 à 10 % en poids d'un dispersant.

2. Procédé selon la revendication 1, dans lequel la transmission est une transmission automatique.

3. Procédé selon la revendication 1, dans lequel R¹ et R² sont chacun indépendamment des groupes alkyle comportant 8 à 20 atomes de carbone.

4. Procédé selon la revendication 1, dans lequel l'amine tertiaire est un produit dérivé de dicocoalkylamine.

5. Procédé selon la revendication 1, dans lequel R³ est un groupe alkyle contenant un polyol.

6. Procédé selon la revendication 1, dans lequel l'amine de (b) est représentée par la formule
R¹R²N-CH₂-CHOH-CH₂OH
dans laquelle R¹ et R² sont chacun indépendamment des groupes alkyle comportant d'environ 8 à environ 20 atomes de carbone.

7. Procédé selon la revendication 1, dans lequel l'amine de (b) comprend le produit réactionnel de dicocoamine et d'une ou plusieurs moles de 2,3-époxy-1-propanol ou de 3-chloropropane-1,2-diol.

8. Procédé selon la revendication 1, dans lequel le dispersant comprend un dispersant succinimide.

9. Procédé selon la revendication 1, dans lequel le lubrifiant comprend en outre au moins un additif sélectionné dans le groupe constitué de détergents, d'antioxydants, d'agents de gonflement des joints d'étanchéité, d'agents anti-usure, et de modificateurs de frottement.

10. Procédé selon la revendication 1, dans lequel le lubrifiant comprend en outre au moins un additif sélectionné dans le groupe constitué d'esters de borates organiques, de sels de borates organiques, d'esters de phosphores organiques, de sels de phosphores organiques, d'acides de phosphores inorganiques, et de sels de phosphores inorganiques.
